

## UNITED STATES PATENT OFFICE

1,927,160

## PROCESS FOR THE COLORATION OF CELLULOSE ESTER AND ETHER MATERIALS

George Holland Ellis and William Bertram Miller, Spondon near Derby, England, assignors to Celanese Corporation of America, a corporation of Delaware

No Drawing. Application January 29, 1930,  
Serial No. 424,442, and in Great Britain  
February 23, 1929

12 Claims. (Cl. 8—5)

This invention relates to the coloring of textile materials made of or containing cellulose acetate or other esters of cellulose, or made of or containing cellulose ethers.

- 5 The coloration of textile materials can be effected, as is known, by the oxidation thereon of various oxidizable aromatic amines. Full and fast black shades have long been produced on cellulosic materials in this manner. To obtain 10 satisfactory results, particularly when employing aniline, it has usually been regarded as good practice not only to avoid the presence of free acid but to have part of the aromatic amine present in the free state; tendering of the fibres is also avoided 15 thereby. When the coloration of materials made of cellulose esters or ethers is attempted in this way it is found that the oxidation of the aromatic amine on the material does not proceed so readily as is the case on cellulosic materials.
- 20 It has now been found that the conditions requisite for the production of satisfactory colorations on cellulose ester or ether materials by the oxidation of aromatic amines, particularly aniline, thereon are essentially different from 25 those which yield the best results in the case of cellulosic materials and that the coloration of cellulose ester or ether materials by this method is much facilitated by the presence of acid in considerably greater proportions than those commonly employed in the coloration of cellulosic 30 materials by similar methods.

According to this invention colorations are produced on materials made of cellulose acetate or other cellulose esters, or made of cellulose ethers, 35 by the oxidation thereon of aromatic amines in the presence of mineral acid in quantity chemically equivalent thereto, there being present in addition a quantity of a substance having an acid reaction, for example a mineral or organic acid, or an acid salt, or a salt having an acid reaction, 40 but preferably an organic acid.

The process is of particular advantage when it is required to color cellulose ester and ether materials by the oxidation thereon of comparatively 45 difficultly oxidizable amines, for example aniline, but the invention is not limited to the use of such amines. In place of aniline there may be employed any other aromatic amine capable of yielding colorations upon oxidation on textile materials, e. g. 1-naphthylamine, a diamino-diphenylamine, p - aminodiphenylamine, dianisidine, benzidine, or tolidine, or a mixture of two or more 50 of such aromatic amines.

In carrying the invention into effect the aromatic amine and equivalent quantity of mineral

acid may conveniently be applied to the materials in the form of the mineral acid salts of the amine. The materials may, for example, be padded with a solution or liquor containing a mineral acid salt of aniline, e. g. the hydrochloride or nitrate, a substance having an acid reaction, e. g. acetic acid or a salt having an acid reaction such as aluminium chloride, and an oxidizing agent, for example a chlorate with or without oxidation catalysts such as salts of vanadium, copper, or iron. After padding and drying the materials may be aged and may then be chromed and soaped according to the usual methods. Full "ungreenable" black shades are obtained by oxidizing aniline in this manner on cellulose acetate 60 materials.

The invention is not limited however to the application of the aromatic amine salt, acid, and oxidizing agent by padding, nor to the application of these materials in a single operation. For example they may be applied by printing or other means of local application or by a simple passage of the material through a bath containing them or they may be applied in succession by padding the material with, or passing the material through, two or more solutions each containing one or more of the necessary compounds.

When dyeing cellulose ester or cellulose ether materials according to the above process, white or coloured pattern effects may be simultaneously produced thereon. White pattern effects for example may be produced on a black or coloured ground by local application, at an appropriate stage of the process, of a "resist" or "discharge" preparation, that is to say, a preparation consisting of or containing an agent which inhibits, either mechanically or chemically, the oxidation of the aniline or other aromatic amine or amines, for example a reducing agent or an agent which neutralizes acids or which substitutes organic acid for mineral acid, e. g. sodium formaldehyde sulphoxylate, zinc oxide, sodium or potassium acetate, or sodium sulphocyanide. The "resist"-or "discharge" preparations may contain, in addition to the agent which inhibits oxidation of the aromatic amine, suitable thickening agents to render them suitable for application by printing or other mode of local application. Thus white "resist" or "discharge" effects on a dark ground may be obtained on cellulose ester or ether materials by printing or otherwise locally treating them with the "resist" or "discharge" preparation, drying, and then applying a solution containing an aromatic amine mineral acid salt, an acid substance, and an oxidizing agent; or the 70 75 80 85 90 95 100 105 110

latter solution may be applied first and the material dried and printed or otherwise locally treated with the "resist" or "discharge" preparation; upon ageing the material the oxidation coloration is only developed upon the parts which have not been treated with the "resist" or "discharge" preparation. Alternatively the order of the operations may be that described in U. S. patent application S. No. 383,977, filed August 6, 1929, that is to say the material may be impregnated with an oxidizing agent, printed or otherwise locally treated with a "resist" preparation comprising a reducing agent, then padded with a solution containing a mineral acid salt of an oxidizable aromatic amine and free acid, and finally aged and finished in the usual manner. Colored pattern effects may be obtained in a similar manner by incorporating in the aforesaid "resist" or "discharge" preparations dye-stuffs which have affinity for cellulose esters or ethers and which are unaffected by the "resist" or "discharge" preparations or by the ageing and finishing processes.

Though the invention has been more particularly described with reference to the coloring of materials made of cellulose acetate it is also applicable to the coloring of materials made of other cellulose esters, for example cellulose formate, propionate, or butyrate, or the products obtained by the treatment of alkalinized cellulose with esterifying agents (e. g. the product known as "immunized cotton" obtained with p-toluenesulphochloride) or of cellulose ethers, for instance methyl, ethyl, or benzyl cellulose or the corresponding condensation products of cellulose and glycols or other polyhydric alcohols, or made of mixtures of two or more of these products.

The invention may also be applied to the dyeing or otherwise coloring of materials containing one or more cellulose esters or ethers in admixture with a material or materials of another kind, particularly animal fibres such as wool or natural silk. A material containing cellulose acetate and wool may for example be dyed in a solid black or other shade according to the process of the invention.

The invention is illustrated but not limited by the following examples:—

#### 50 Example 1

A fabric woven from cellulose acetate yarns is treated in a suitable padding machine with a pad liquor composed as follows:

|    |                       |       |
|----|-----------------------|-------|
| 55 | Solution A            | Grams |
|    | Aniline hydrochloride | 127   |
|    | Glacial acetic acid   | 25    |
|    | Water                 | 248   |
|    | Alcohol               | 100   |
| 60 | Gum arabic 1:1        | 200   |
|    |                       | 700   |

|    |                 |       |
|----|-----------------|-------|
| 65 | Solution B      | Grams |
|    | Sodium chlorate | 80    |
|    | Cupric chloride | 3     |
|    | Water           | 217   |
|    |                 | 300   |

70 Solutions A and B are mixed just before use. The padded material, which is squeezed to hold about its own weight of liquor, is dried either in a hot flue or on heated cylinders, after which it is given a passage through the "rapid ager" for 75 minutes at 100° C. After ageing, the material

is run through a bath of sodium bichromate, 5 gms. per litre, at 50° C. for two minutes, rinsed, soaped or further treated as desired or requisite. A good full black shade is thus obtained.

80

#### Example 2

A woven fabric composed of cellulose acetate is printed on a roller printing machine or by hand block with a four color design using four printing colors as follows:—

|     |                   |      |
|-----|-------------------|------|
| (a) | Grams             |      |
|     | Gum arabic 1:1    | 470  |
|     | Methylated spirit | 50   |
|     | Water             | 180  |
|     | Sodium acetate    | 300  |
|     |                   | 1000 |

|     |                                           |      |
|-----|-------------------------------------------|------|
| (b) | Grams                                     |      |
|     | Rhodamine 6G powder (Color Index No. 752) | 95   |
|     | Methylated spirit                         | 40   |
|     | Water                                     | 50   |
|     | Sodium acetate                            | 160  |
|     | Gum arabic 1:1                            | 300  |
|     |                                           | 450  |
|     |                                           | 1000 |

|     |                                                                      |      |
|-----|----------------------------------------------------------------------|------|
| (c) | Grams                                                                |      |
|     | 3:3'-dinitro - 4:4' - diamino - diphenyl - methane 20% aqueous paste | 100  |
|     | Methylated spirit                                                    | 105  |
|     | Water                                                                | 50   |
|     | Sodium acetate                                                       | 100  |
|     | Gum arabic 1:1                                                       | 300  |
|     |                                                                      | 450  |
|     |                                                                      | 110  |
|     |                                                                      | 1000 |

|     |                                            |      |
|-----|--------------------------------------------|------|
| (d) | Grams                                      |      |
|     | 1:4 dimethyldiaminoanthraquinone 20% paste | 100  |
|     | Methylated spirit                          | 50   |
|     | Water                                      | 115  |
|     | Sodium acetate                             | 100  |
|     | Gum arabic 1:1                             | 300  |
|     |                                            | 450  |
|     |                                            | 1000 |
|     |                                            | 120  |

The printed fabric, having been dried as usual, is treated in a suitable padding machine with the aniline black liquor described in Example 1, the fabric passing through the padding rollers with out being drawn through the liquor. After drying the material is given a passage through the "rapid ager" and is then steamed in the "cottage steamer" for  $\frac{1}{2}$  to 1 hour with steam at 5 lbs. pressure. The subsequent operations of chroming and soaping are carried out as in Example 1, after which the fabric is further treated as desired or requisite. A pattern in white, red, yellow and blue on a black ground results.

135

#### Example 3

A fabric woven from cellulose acetate yarns is treated in a suitable padding machine with a pad-liquor composed as follows:—

|    |                                    |       |
|----|------------------------------------|-------|
| 75 | Solution A                         | Grams |
|    | Aniline hydrochloride              | 96    |
|    | p-aminodiphenylamine hydrochloride | 52    |
|    | Glacial acetic acid                | 25    |
|    | Water                              | 145   |
|    | Alcohol                            | 227   |
|    | Gum arabic 1:1                     | 100   |
|    |                                    | 200   |
|    |                                    | 700   |
|    |                                    | 150   |

|                 |       |
|-----------------|-------|
| Solution B      | Grams |
| Sodium chlorate | 80    |
| Cupric chloride | 3     |
| Water           | 217   |
|                 | —     |
| 5               | 300   |

Solutions A and B are mixed just before padding. The material is impregnated with this mixture, squeezed to hold its own weight of liquor and dried. It is then given a five minutes' passage through the "rapid ager" after which it is chromed in a 1/2% solution of sodium dichromate for 2 minutes at 50° C., rinsed, soaped or otherwise treated as desired or requisite. A fast black 15 results.

*Example 4*

A woven fabric composed of cellulose acetate 20 yarns is treated in a suitable pad mangle with a pad liquor of the following composition:—

|                         |       |
|-------------------------|-------|
| Benzidine hydrochloride | Grams |
| Acetic acid conc.       | 56    |
| Methylated spirit       | 25    |
| Cupric chloride         | 100   |
| Sodium chlorate         | 4     |
| Water                   | 80    |
|                         | 735   |
| 30                      | —     |
| 1000                    |       |

The material after padding so that it holds its own weight of pad liquor, is dried either in a flue with hot air or on heated drying cylinders and is then given a passage of five minutes through the 35 "rapid ager" at 100° C., after which it is rinsed and soaped or otherwise treated as desired or requisite. The cellulose acetate is thus colored a deep brown shade.

*Example 5*

A fabric composed of cellulose acetate yarns is padded in a 5% solution of sodium chlorate and dried. It is then printed with a printing paste 45 composed as follows:—

|                                |       |
|--------------------------------|-------|
| Gum arabic 1:1                 | Grams |
| China clay                     | 260   |
| Zinc formaldehyde sulphoxylate | 100   |
| 50 Water                       | 200   |
|                                | 440   |
| 1000                           | —     |

The printed fabric is dried and steamed in the 55 "cottage steamer" for 3 minutes at 5 lbs. pressure or in the "rapid ager" for an equivalent steaming. It is then padded in a solution of the following composition, being preferably passed straight to the squeezing rollers without previous immersion:—

|                           |       |
|---------------------------|-------|
| Aniline                   | Grams |
| Hydrochloric acid 28° Tw. | 54    |
| Glacial acetic acid       | 80    |
| 65 Methylated spirit      | 15    |
| Cupric chloride crystals  | 60    |
| Gum arabic 1:1            | 2.4   |
| Water                     | 90    |
|                           | 298.6 |
| 70                        | —     |
| 600.0                     |       |

The material after padding is dried and aged in the "rapid ager" at 100° C. or steamed for 5 minutes in the "cottage steamer". It is finally washed off well and soaped. A white pattern on 75 a black ground is obtained.

What we claim and desire to secure by Letters Patent is:—

1. Process for the coloration of materials containing organic derivatives of cellulose, comprising oxidizing an aromatic amine thereon in the presence of a mineral acid in quantity at least sufficient to form a salt with the amine and in the presence of an additional acid reacting substance. 80

2. Process for the coloration of materials containing organic derivatives of cellulose, comprising oxidizing thereon in the presence of an acid reacting substance an aromatic amine in the form of a salt of an inorganic acid. 85

3. Process for the coloration of materials containing organic derivatives of cellulose, comprising oxidizing aniline thereon in the presence of a mineral acid in quantity at least sufficient to form a salt with the aniline and in the presence of an additional acid reacting substance. 90

4. Process for the coloration of materials containing organic derivatives of cellulose, comprising oxidizing aniline thereon in the form of a salt of an inorganic acid and in the presence of an additional acid reacting substance. 95

5. Process for the coloration of materials containing organic derivatives of cellulose, comprising oxidizing aniline thereon in the form of a salt of an inorganic acid and in the presence of an organic acid. 100

6. Process for the coloration of materials containing cellulose acetate, comprising oxidizing thereon in the presence of an acid reacting substance, an aromatic amine in the form of a salt of an inorganic acid. 105

7. Process for the coloration of materials containing cellulose acetate, comprising oxidizing aniline thereon in the presence of a mineral acid in quantity at least sufficient to form a salt with the aniline and in the presence of an additional 110 acid reacting substance. 115

8. Process for the coloration of materials containing cellulose acetate, comprising oxidizing aniline thereon in the form of a salt of an inorganic acid and in the presence of an additional 120 acid reacting substance. 120

9. Process for the coloration of materials made of or containing cellulose acetate, comprising oxidizing aniline thereon in the presence of a mineral acid in quantity at least sufficient to 125 form a salt with the aniline and in the presence of an organic acid. 125

10. Process for the coloration of materials containing cellulose acetate comprising oxidizing aniline thereon in the form of aniline hydrochloride and in the presence of acetic acid. 130

11. Process for the coloration of materials containing organic derivatives of cellulose which comprises oxidizing aniline thereon with the aid of a chlorate in the presence of a mineral acid in quantity at least sufficient to form a salt with the aniline and in the presence of an additional acid reacting substance, the color formation being effected by ageing or steaming. 135

12. Process for the coloration of materials made of or containing cellulose acetate, which comprises oxidizing aniline thereon with the aid of a chlorate in the presence of a mineral acid in quantity sufficient to form a salt with the aniline and in the presence of an organic acid 140 the color formation being effected by ageing or steaming. 145

GEORGE HOLLAND ELLIS.  
WILLIAM BERTRAM MILLER. 150